

## UNITED STATES PATENT OFFICE

2,504,717

## REVERSIBLE LUBRICATING GREASE COMPOSITION

Arnold J. Morway, Clark, and John C. Zimmer,  
Union, N. J., assignors to Standard Oil Develop-  
ment Company, a corporation of Delaware.

No Drawing. Application September 20, 1947,  
Serial No. 775,370.

6 Claims. (Cl. 252—39)

1.

The present invention relates to a reversible lubricating grease composition, particularly reversible greases which are water resistant, transparent, mechanically and thermally stable and adapted for use in "lubricated for life" bearings. Reversible greases are those grease compositions which can be heated to above their melting point and cooled without the loss of their grease structure. This application is a continuation in part of application Serial No. 414,644, filed October 10, 1944, now abandoned.

There are numerous types of grease compositions in common usage and of these numerous types each will be found to vary greatly in composition although fundamentally they consist of soap mixed with ordinary lubricating oil. Both the oil and the type and quantity of soap may be widely varied to meet the conditions of a particular lubrication problem requiring the use of a semi-fluid lubricant. The lubrication problems to which the grease compositions are applied are almost as numerous as the compositions themselves. One troublesome problem presents itself with the attempt to lubricate bearings operated at temperatures in the neighborhood of the boiling point of water and often above and especially those bearings which operate at temperatures between 140° F. and 200° F. in the presence of water. Greases, for the most part, are either dispersions or solutions of metallic soaps in a mineral lubricating oil which will range in viscosity from 60 seconds Saybolt at 100° F. for the light oils to about 4500 seconds Saybolt at 100° F. for the bright stocks. The soaps ordinarily used for the making of greases consist of the alkali metal soaps, alkaline earth soaps, or mixtures thereof. Sometimes special soaps such as aluminum soaps are employed. In the preparation of the soaps an excess of the metal is sometimes employed which results in the production of a basic soap. In the lubrication of bearings operating at temperatures above 140° F. the ordinary type greases are found to have many imperfections. For instance, the lime soap greases require the presence or incorporation of a small amount of water in the composition to secure the grease-like structure. When temperatures around 212° F. are obtained the water present in a lime soap grease evaporates and the lime soap, which is insoluble in the oil precipitates out and the composition is converted into a layer of soap and a layer of mineral oil with no grease structure involved. Alkali metal soaps are readily water soluble and when greases containing such alkali metal soaps are used in

the presence of water they are soon dissolved out and removed from the bearing. With the removal of the soap, which functions to hold the oil, the oil is no longer retained in the bearing.

It has previously been suggested that greases might be prepared from barium soaps. In the prior art, however, difficulty has been encountered in preparing stable soaps of barium base and it has been held generally that only the basic barium soaps, i. e., those containing an excess of barium hydroxide, could be used to prepare greases. Basic barium soap greases, although possessing relatively high melting points, often reaching as high as 400° F., depending upon the amount and kind of basic barium soap present in the oil, lose their grease structure when subjected to temperatures in the neighborhood of their melting point and revert to a mixture of stratified oil and soap. After the melting point of a basic barium soap grease has been reached the only means of retaining the grease-like structure is to work the grease while it cools.

Some efforts have been made in the prior art to improve the mechanical stability of barium soap greases by incorporating certain stabilizers, but in general it has been considered necessary to use an excess of the barium compound, even when special stabilizers are added. The present invention includes as one aspect a method of preparing a mechanically stable grease having the otherwise desirable properties of barium base greases without using an excess of the barium oxide or hydroxide with its accompanying disadvantages.

Mixed alkaline earth soap greases such as the calcium-barium greases possess the faults of both lime soap greases and the basic barium soap greases. Aluminum soap greases although often used in life-time bearings, tend to emulsify with water or become semifluid and rubbery at elevated temperatures, such as above 140° F. and for these reasons cannot be retained in a bearing operating under such conditions. Since the retention of fluid oil in a bearing offers mechanical problems, it is apparent that the greases as above described are not particularly adaptable to the lubrication of life-time bearings and that an improved grease devoid of these imperfections is especially desirable.

The principal object of this invention is the development of a barium soap grease of excellent structure, easy to prepare and which is reversible, water resistant, transparent and mechanically and thermally stable. These and other objects

will be apparent to those skilled in the art upon reading the following description.

A further object of this invention is to compound barium soap greases in a manner which avoids the introduction of objectionable ingredients which appear to have given rise to difficulties encountered in prior art attempts to prepare barium base greases.

It has now been discovered that greases compounded of neutral and/or acid barium soaps and mineral lubricating oils produce greases which are water insoluble, transparent, mechanically and thermally stable and reversible, provided certain procedures are observed during their preparation. These greases can be used at any temperature up to 212° F. in the presence of water without decomposition and at temperatures above the boiling point of water, not to exceed the ignition or decomposition temperature of the constituents themselves, and may be liquefied and solidified innumerable times without the loss of lubricating quality or grease structure.

It appears that two special procedures are desirable in the preparation of mechanically stable barium greases having the other desirable properties mentioned above. In the first place it appears to be desirable to avoid the introduction of barium carbonate when the barium oxide or hydroxide is used as a saponifying agent. Apparently commercial barium oxide, or hydroxide, tends to react with carbon dioxide in the air over a period of time to revert to the somewhat more stable carbonate. If a barium oxide which includes an appreciable quantity of the carbonate is employed in forming the grease, or in forming the soap to be incorporated in grease, the difficulties known to the prior art in securing proper grease structure, mechanical stability, reversibility, etc., appear to arise. Hence it is desirable to use either a freshly calcined barium oxide (or freshly hydrated oxide which has been kept away from the air since calcination) or to keep the calcined barium oxide in an inert atmosphere, for example in a nitrogen atmosphere, after calcination.

A further requisite which appears to be quite essential to securing a good stable, reversible grease structure, appears to be the formation of the soap, or the saponification of fatty material, directly in the mineral oil which is to serve as the liquid lubricating element of the finished grease composition. The use of preformed soap has been found to be unsatisfactory and in fact it is commonly impossible to secure a grease structure at all when it is attempted to incorporate a preformed barium soap into lubricating oil. This is particularly true with respect to the basic barium soaps used in the prior art.

A still further distinctive aspect of the present invention is, as suggested above, the preparation of a neutral or slightly acid barium soap grease, as distinguished from the basic barium greases known to the prior art. The advantages of reversibility, improved texture and general stability referred to more fully below appear to be derived largely from the elimination of excess barium oxide or hydroxide which was commonly considered essential in the prior art. Hence the quantity of saponification agent preferably should not exceed stoichiometrical proportions.

Preferably, the barium oxide employed is freshly calcined by heating barium carbonate, or the impure oxide, to a sufficient temperature to drive off the carbon dioxide. Barium carbonate is not easily decomposed but the calcination appears

to be facilitated by the addition of a small amount of carbon such as charcoal, carbon black or other carbonaceous materials, with heating to a fairly high temperature. In the absence of carbon or carbonaceous materials, it may be necessary to heat the carbonate to a temperature as high as 1350° C. if heating is carried out under atmospheric pressure. By using reduced pressures, and/or an atmosphere free from carbon dioxide, the temperature may be somewhat lower. In any case heating is carried out at a sufficiently elevated temperature and over a period sufficiently extended to decompose substantially all of the carbonate and obtain a substantially pure oxide.

As suggested above, if the calcined oxide is not to be used promptly, it should be protected from access to air, preferably by storing it in a nitrogen atmosphere.

The barium oxide, preferably substantially free from the carbonate as mentioned above, may be hydrated to the hydroxide, preferably in an inert medium such as oil, before adding the fatty material and mineral oil, or it may be added as an aqueous slurry to the soap stock in mineral oil solution. However, a fairly pure commercial barium hydroxide appears to be satisfactory although it is preferred to use the freshly hydrated oxide. Conventional methods for grease manufacture may be employed with the exception and the added advantage that after the soaps are completely formed and dispersed in the mineral oil the grease may be placed in final package containers and permitted to cool without the necessity of further working.

Preferably, the soap stock or fatty material is first dissolved by stirring it into at least a portion and preferably all of the lubricating oil, accompanied by heating, if necessary, to a temperature at least equal to the melting point of the soap stock. Thereafter, for a neutral soap grease the stoichiometrical proportions of hydrated barium oxide are added, or slightly less if an acid grease is desired. During the formation of the soap, the ingredients are heated moderately, e. g., to a temperature around 200° F. Thereafter, in order to remove the water, the temperature is raised to a range of about 275° F. to 425° F., preferably 300° to 400° F., to obtain a clear solution, further mineral oil is added with stirring, if necessary, and the grease is poured into containers to cool. Such containers preferably may be the final shipping containers to avoid further handling.

The total amount of soap in the grease made in accordance with this invention will range from about 5% to about 50% by weight based upon the total grease composition depending upon the properties desired in the finished grease, the type and viscosity of the oil used and the character of the fat or acid employed in the production of the soap.

Although a wide range of lubricating oils may be employed as the lubricant in the grease, in general the base oil comprises an oil having a S. U. V. in the range of from about 35 to 220 seconds at 210° F. However, for the production of most greases of the type contemplated by this invention it is preferred to use a base oil having a viscosity of from 100 to 2400 at 100° F.

The usual types of soap stocks, such as animal or vegetable fats or commercial stearic, palmitic, and oleic acids, as well as fatty acids split from hydrogenated fats such as hydrogenated fish oil acids, which soap stocks contain at least 12 carbon atoms to the molecule, usually 12 to 22 or 24

## 5

carbon atoms, may be used for the production of the soaps useful for the purposes of this invention. Other additives such as anti-oxidants, adhesives and rust-preventing agents may be incorporated without departing from the scope of this invention.

The following examples will serve as illustrations of typical compositions according to this invention:

## Example 1

10.00% by weight commercial oleic acid.  
8.07% by weight barium hydroxide-oil mixture.  
81.93% by weight lubricating oil (low cold test coastal type oil).  
<sup>1</sup> 33 1/3% water, 33 1/3% calcined barium oxide, 33 1/3% low cold test naphthenic type oil.

The oleic acid and the homogeneous emulsion of barium hydroxide and oil are added together with about 1/4 of the lubricating oil. The mixture is heated for a short time at 200° F., with stirring, and the remainder of the mineral oil is added. The product is next allowed to cool substantially to room temperature where it sets up as a smooth cup grease and is later reheated to about 300° F. until all water is driven off. The grease is then poured into containers and permitted to cool. The finished grease is transparent and smooth, has a melting point of 240° F., a penetration of 320/340 at 77° F. and may be alternately melted and cooled without loss of structure.

## Example 2

A harder grease was prepared by the same general method as that in Example 1 using the following ingredients. Percentages given are by weight, as in Example 1.

20% commercial oleic acid.  
19% barium hydroxide-oil mixture.  
61% lubricating oil (low cold test coastal).

<sup>1</sup> 28.5% calcined barium oxide, 28.5% water, 43.0% lubricating oil.

An excellent hard grease resulted which ran for 1 hour in the Annular Bearing Engineer's Committee test machine at temperatures above 230° F. with no leakage and with good lubrication. The grease showed some tendency to ball up and to become somewhat brittle at temperatures above 200° F. This grease, which contains less mineral oil than that of Example 1, appears to be particularly suitable where a hard grease is needed for service at moderate temperatures.

## Example 3

The grease of Example 2 was modified by incorporating additional oil and a small amount of an aluminum soap. Thus 2 grams of aluminum stearate were slurried with 48 grams of mineral lubricating oil and the slurry was added to 200 grams of the grease. The mixture was heated to the melting point and thereafter cooled slowly. An excellent product of homogeneous structure was obtained.

## Example 4

20.00% hydrogenated fish oil acids  
19.00% barium hydroxide-oil mixture.  
61.00% low cold test coastal type lubricating oil

<sup>1</sup> 28.5% calcined barium oxide, 28.5% water, 43.0% lubricating oil.

The grease was made according to the procedure outlined in Example 1 above, resulting in a product having a penetration of 265/280 at 77° F. and a melting point of 250° F. The char-

## 6

acter and properties of this grease can be altered somewhat by lowering the fabrication temperature to below 200° F. By compounding this composition at the lower temperature a grease is formed which contains considerable water and on heating to over 210° F. steaming and bubbling occur. However, when again cooled to below the boiling point of water the grease will return to a smooth homogeneous lubricant.

- 10 With reference to the barium compounds, it appears that the calcined barium oxide is much more active than commercial barium hydroxide, probably because of the presence of perceptible quantities of barium carbonate in the latter.  
15 For this reason it is preferred to hydrate the oxide freshly in the absence of carbon dioxide. The hydration in oil, as suggested above, is a convenient way to exclude carbon dioxide but there are various other ways of excluding it, as  
20 will be apparent to those skilled in the art. It appears to be desirable to use an excess of water in hydrating and, as indicated above, the resulting soap is preferably neutral or slightly acid, i.e. pH at least as low as 7.0.  
25 The expression "consisting essentially," as used in the claims, means that the composition is made up substantially entirely of the ingredients recited and that such ingredients are the main ones and those which characterize the composition. This does not exclude minor quantities of other conventional ingredients which are relatively inert or are of such nature and/or present in such small quantities that the essential properties of the composition are substantially un-  
30 affected.

While specific procedures and temperatures have been recited in the foregoing examples, it will be understood that these may be varied somewhat. Slow cooling of the barium greases appears to be essential; hence the process is not as satisfactorily conducted with fast cooling continuous process apparatus. Otherwise the continuous process appears to be applicable. In general the barium soaps will comprise preferably from 15 to about 35% by weight of the greases, but greases having soap content of 5 to 50% may be prepared satisfactorily. The addition of a small amount of aluminum soap, e.g. aluminum stearate, tends to make a smoother and more homogeneous product. The aluminum soap is preferably employed in proportions of 0.2 to 4% by weight, based on the total composition, but very satisfactory grease may be prepared without its use.

## 55 We claim:

1. An anhydrous, reversible lubricating grease composition consisting essentially of 50 to 90% by weight, based on the total composition, of a low cold test mineral oil thickened to a smooth 60 homogeneous solid grease structure with 10 to 50% of barium soap of fatty acid having 12 to 24 carbon atoms, said barium soap having a pH value at least as low as 7.0 and being prepared by dissolving said fatty acid in said mineral oil, 65 adding an aqueous-oil slurry of carbonate-free barium hydroxide in not more than stoichiometrical proportions, based on the fatty acid, and heating the ingredients to a temperature of about 200° F. to form barium soap in situ.
2. A reversible anhydrous lubricating grease composition consisting essentially of a mineral base lubricating oil thickened to a smooth homogeneous solid grease consistency by 10 to 75 35% by weight, based on the total composition, of barium soap of aliphatic fatty acid having

between about 12 and about 24 carbon atoms, said soap having a pH value at least as low as 7.0, said soap being prepared by dissolving said fatty acid in said oil, adding not more than a theoretical quantity of a carbonate-free barium hydroxide in an aqueous-oil slurry to saponify said acid, heating the ingredients to a temperature of about 200° F. to form the soap in situ, and thereafter heating to a temperature within the range of about 275° to 425° F. to remove water and leave a smooth grease structure.

3. A process for making a reversible lubricating grease composition substantially free of soaps other than barium soap which consisting essentially of the steps of dissolving aliphatic fatty material having between 12 and 24 carbon atoms per molecule in mineral lubricating oil, neutralizing said fatty material with not more than a stoichiometrical quantity of freshly hydrated barium oxide which is substantially free of barium carbonate, heating said composition to a temperature between 275° F. and 425° F., and slowly cooling said composition to a soap forming temperature of about 200° F., and thereafter removing water by heating further to substantially ambient temperature to obtain a smooth homogeneous solid grease product having a pH value not greater than 7.0.

4. A process for preparing a reversible lubricating grease of barium soap and mineral lubricating oil base substantially free of other soaps, which consists essentially of calcining a barium-oxygen compound containing CO<sub>2</sub> to substantially remove said CO<sub>2</sub> and leave a substantially pure barium oxide, hydrating said oxide in a manner substantially to protect said oxide from contact with CO<sub>2</sub>, incorporating said hydrate together with at least a theoretical proportion of C<sub>12</sub> to C<sub>24</sub> fatty acid in mineral base lubricating oil, heating to an elevated temperature to form a nonbasic substantially pure barium soap in situ in said oil, and slowly cooling the oil and soap mixture thereby forming a stable smooth homogeneous solid grease structure.

5. A process for preparing a smooth solid homogeneous reversible lubricating grease of barium soap and mineral oil base substantially free of other soaps, which consists essentially of the steps of mixing a sufficient quantity of saponifiable aliphatic fatty material for forming said solid grease with mineral base lubricating oil when saponified therein, heating said mixture to a saponification temperature, and saponifying said fatty material in situ in said oil by introducing barium hydroxide in quantity not exceeding stoichiometrical proportions, based on said saponifiable material, said barium hydroxide being substantially free of barium carbonate.

6. A process as in claim 5 wherein said barium hydroxide is produced by hydrating barium oxide free of carbon dioxide derivative impurities in a manner to prevent atmospheric access.

ARNOLD J. MORWAY.  
JOHN C. ZIMMER.

#### REFERENCES CITED

The following references are of record in the file of this patent:

#### UNITED STATES PATENTS

| Number    | Name                 | Date           |
|-----------|----------------------|----------------|
| 2,154,383 | Ott et al. -----     | Apr. 11, 1939  |
| 2,303,256 | Camelford -----      | Nov. 24, 1942  |
| 2,332,247 | Morway et al. -----  | Oct. 19, 1943  |
| 2,417,433 | McLennan -----       | Mar. 18, 1947  |
| 2,434,539 | Beerbower et al. --- | Jan. 13, 1948  |
| 2,450,224 | Bergmann et al. ---  | Sept. 28, 1948 |

#### OTHER REFERENCES

Boner: "Metallic Soaps for Thickening Mineral Oils," article in Industrial and Engineering Chemistry, vol. 29, pp. 58, 59, and 60, Jan. 1937.

McLennan: "Methods of Compounding Barium Greases," article in National Petroleum News, R-234, R-236, R-238, R-239, April 5, 1944.